

3,542,655

## ELECTRODEPOSITION OF COPPER

Otto Kardos, Ferndale, Hugh B. Durham, Southfield, Arthur J. Tomson, Novi, and Donald A. Arcilesi, Sterling Township, Utica, Macomb County, Mich., assignors to M&T Chemicals Inc., New York, N.Y., a corporation of Delaware

No Drawing. Filed Apr. 29, 1968, Ser. No. 725,209

Int. Cl. C23b 5/20, 5/46

U.S. Cl. 204—52

33 Claims

## ABSTRACT OF THE DISCLOSURE

According to certain of its aspects, this invention relates to novel compositions and to a process for electrodepositing bright, strongly leveled, ductile copper from an aqueous acidic copper plating bath containing chloride ions and at least one member from each of the following groups:

(1) a polysulfide compound of the formula



(2) a heterocyclic compound of the formula



and/or tautomers thereof; and

(3) a polyether, containing at least 5 ether oxygen atoms per molecule;

wherein each R is independently a divalent aliphatic or aromatic non-heterocyclic group of 1-10 carbon atoms; R' is hydrogen, a metal cation, a monovalent aliphatic or aromatic organo group of 1-20 carbon atoms, or the groups  $-R-SO_3 M$  or  $-R-(S)_q-RSO_3 M$  wherein q is an integer 2-5; M is a cation;



R'' is hydrogen or an alkyl, hydroxyalkyl or aminoalkyl group of 1-6 carbon atoms; Y is a divalent organo group of 1-10 carbon atoms which forms a 5-6-membered cyclic ring structure with the group



and n is an integer 2-5 inclusive.

This invention relates to novel processes and compositions for the electrodeposition of copper from aqueous acidic baths. More particularly, this invention relates to certain bath compositions containing specified combinations of chemical ingredients and to the use of such compositions to obtain bright, ductile, strongly leveled copper electrodeposits.

It is an object of this invention to obtain bright, ductile, leveled copper electrodeposits. A further object of the invention is to provide novel plating bath compositions from which bright copper electrodeposits may be obtained wherein said electrodeposits exhibit good leveling and ductility over wide current density ranges. Other objects of the invention will be apparent from the following detailed description.

In accordance with certain of its aspects, this invention relates to novel compositions and to a process for electrodepositing bright, strongly leveled, ductile copper from an aqueous acidic copper plating bath containing chloride ions and at least one member from each of the following groups:

(1) a polysulfide compound of the formula



(2) a heterocyclic compound of the formula



and/or tautomers thereof; and

(3) a polyether, containing at least 5 ether oxygen atoms per molecule;

wherein each R is independently a divalent aliphatic or aromatic non-heterocyclic group of 1-10 carbon atoms; R' is hydrogen, a metal cation, a monovalent aliphatic or aromatic organo group of 1-20 carbon atoms, or the groups  $-R-SO_3 M$  or  $-R-(S)_q-RSO_3 M$  wherein q is an integer 2-5; M is a cation;



20 R'' is hydrogen or an alkyl, hydroxyalkyl or aminoalkyl group of 1-6 carbon atoms; Y is a divalent organo group of 1-10 carbon atoms which forms a 5-6-membered cyclic ring structure with the group



25 and n is an integer 2-5 inclusive.

When several radicals R are present, the R groups may or may not be identical. As used herein, the term "leveled" denotes a surface which is smoother than its substrate.

The combination of these three additives in a chloride-containing copper plating bath gives unexpected beneficial effects over the use of each additive alone in a chloride-containing copper plating bath.

30 Simultaneous use of at least one member from each of the three groups of additives gives bright copper deposits over a wide current density range with strong leveling properties. The high degree and rate of leveling leads to an important economy in finishing costs and materials.

35 The improved low current density brightness (i.e. the widening of the bright current density range) is important if strongly profiled objects are to be plated. The polysulfide sulfonates, as defined herein, have been found to be much more effective when employed according to the invention than the corresponding monosulfides.

40 When used alone these additives may be found to be deficient in that the copper deposits obtained may not be bright, smooth, and exhibit adequate leveling properties over a sufficient current density range. Combinations utilizing two of the additives may give fairly bright copper deposits, but the current density range of brightness may be limited and/or the rate of leveling (decrease of surface roughness) may be low. Other double combinations may give striated deposits and limited bright current density ranges.

45 The novel compositions of the invention may be employed in combination with aqueous acidic copper plating baths. Typical aqueous acidic copper plating baths which may be employed in combination with the novel compositions of the invention include the following:

### TABLE I

#### Sulfate bath

- 65 (1)  $CuSO_4 \cdot 5H_2O$ , 150-300 g./l. (preferably about 220 g./l.)  
 $H_2SO_4$ , 10-110 g./l. (preferably about 60 g./l.)  
 $Cl^-$ , 5-100 mg./l. (preferably about 20-40 mg./l.)
- 70 (2)  $Cu(BF_4)_2$ , 100-600 g./l. (preferably about 224 g./l.)  
 $HBF_4$ , 1-60 g./l. (preferably about 3.5 g./l.)

#### Fluoroborate bath

$H_3BO_3$ , 0-30 g./l. (preferably about 15 g./l.)  
 $Cl^-$ , 5-100 mg./l. (preferably about 20-40 mg./l.).

The basis metals which may be electroplated in accordance with the process of this invention may include ferrous metals, such as steel, iron, etc. bearing a surface layer of nickel or cyanide copper; zinc and its alloys including zinc-base die-cast articles bearing a surface layer of cyanide copper or pyrophosphate copper; nickel, including nickel alloys with other metals such as cobalt-iron; aluminum, including its alloys, after suitable pretreatment, etc.

After the deposition of the bright leveled copper deposit of this invention, generally a bright nickel deposit and a chromium deposit (which may be microporous or microcracked) may be applied. The bright acid copper deposit of this invention contributes to the appearance and performance of the composite coating because of its very high rate of leveling, its excellent pore-filling capacity, its high luster, good ductility and low internal stress. It improves corrosion resistance and permits economy in nickel.

Because of its strong leveling properties, its very good performance at high current densities, and its very good mechanical properties the bright acid copper electrodeposits of this invention may be used for industrial applications such as the plating of printing rolls, memory drums, etc., and for electroforming. It gives very good results also for the plating of non-conducting materials, such as plastics, after the usual pretreatment.

The plating conditions for electrodeposition from the aforementioned baths may, for example, include temperatures of 10° C.-60° C. (preferably 20° C.-40° C.); pH (electrometric) of less than about 1.5; and a cathode current density of .1-30.0 amperes per square decimeter (a./s.d.).

Typical average current densities may be 2-20 a./s.d. for the sulfate bath, and about 4-40 a./s.d. for the fluoborate bath. Air agitation, volume agitation, or mechanical agitation may increase the effective current density ranges and enhance the uniformity of the copper deposit.

In accordance with certain of its aspects, this invention relates to novel compositions and to a process for electrodepositing bright, strongly leveled, ductile copper from an aqueous acidic copper plating bath containing chloride ions and at least one member from each of the following groups:

(1) a polysulfide compound of the formula



(2) a heterocyclic compound of the formula



and/or tautomers thereof; and

(3) a polyether, containing at least 5 ether oxygen atoms per molecule;

wherein each R is independently a divalent aliphatic or aromatic non-heterocyclic group of 1-10 carbon atoms; R' is hydrogen, a metal cation, a monovalent aliphatic or aromatic organo group of 1-20 carbon atoms, or the groups  $-R-SO_3M$  or  $-R-(S)_q-RSO_3M$  wherein q is an integer 2-5; M is a cation;



R'' is hydrogen or an alkyl, hydroxyalkyl or aminoalkyl group of 1-6 carbon atoms; Y is a divalent organo group of 1-10 carbon atoms which forms a 5-6-membered cyclic ring structure with the group



and n is an integer 2-5, inclusive.

Sulfide compounds wherein n is an integer 2-4 are preferred. R may be a divalent hydrocarbon group (including such hydrocarbon groups containing inert substituents such as hydroxyl, alkoxy, polyoxyalkylene, halogen, etc.) of 1-10 carbon atoms such as an alkylene group of 1-10 carbon atoms (i.e.,  $-CH_2-$ ,  $-CH_2CH_2-$ ,  $-(CH_2)_3-$ ,  $-(CH_2)_4-$ ,  $-(CH_2)_5-$ , and, in general,  $-(CH_2)_p-$  wherein p is an integer 1-10). R may be a divalent non-heterocyclic group of 1-10 carbon atoms containing 1-3 oxygen, 1-3 sulfur, or 1-3 nitrogen atoms (such as  $-CH_2CH_2OCH_2CH_2-$ ,



In the compound



R' may be a hydrocarbon radical preferably selected from the group consisting of alkyl, alkenyl, alkynyl, cycloalkyl, aralkyl, aryl, alkaryl, including such radicals when inertly substituted. When R' is alkyl, it may typically be straight chain alkyl or branched alkyl, including methyl, ethyl, n-propyl, isopropyl, n-butyl, isobutyl, sec-butyl, tert-butyl, n-amyl, neopentyl, isoamyl, n-hexyl, isohexyl, heptyl, octyls, decyls, dodecyls, tetradecyl, octadecyl, etc. Preferred alkyl includes lower alkyl, i.e., having less than about 8 carbon atoms, i.e., octyls and lower. When R' is alkenyl, it may typically be vinyl, allyl, methallyl, buten-1-yl, buten-2-yl, buten-3-yl, penten-1-yl, hexenyl, heptenyl, octenyl, decenyl, dodecenyl, tetra-deceny, octadecenyl, etc. When R' is alkynyl, it may typically be ethynyl, propargyl, butynyl, etc. When R' is cycloalkyl, it may typically be cyclopentyl, cyclohexyl, cycloheptyl, cyclooctyl, etc. When R' is aralkyl, it may typically be benzyl,  $\beta$ -phenylethyl,  $\alpha$ -phenylpropyl,  $\beta$ -phenylpropyl, etc. When R' is aryl, it may typically be phenyl, naphthyl, etc. When R' is alkaryl, it may typically be tolyl, xylyl, p-ethyl-phenyl, p-nonylphenyl, etc. R' may be inertly substituted, e.g., may bear a non-reactive substituent such as alkyl, aryl, cycloalkyl, aralkyl, alkaryl, alkenyl, ether, etc.

Polysulfide compounds of the formula (1) may typically be prepared by the reaction of an alkali metal salt of a hydropolysulfide and a sultone according to the reaction:



wherein R, R', M, and n are as previously defined.

Specific illustrative reactions may include the following reactions wherein all unsubstituted carbon atoms are attached to hydrogen atoms:





Other preparative reactions which may be used to produce the sulfide compounds employed according to the invention include the direct sulfonation of an organo polysulfide (i.e. direct sulfonation of diphenyl disulfide, ditolyl disulfide, etc.). The polysulfide compounds also may be prepared by the reaction of epichlorohydrin and an alkali metal bisulfite followed by reaction with a poly-

6 sulfide (such as  $\text{Na}_2\text{S}_2$ ,  $\text{R}'\text{S}_2\text{H}$ ,  $\text{R}'\text{S}_2\text{Na}$ , wherein  $\text{R}'$  is as previously defined).

Other preparative reactions may include the following:

- (a)  $\text{SCl}_2 + 2\text{NaS}(\text{CH}_2)_3\text{SO}_3\text{Na} \rightarrow \text{NaO}_3\text{S}(\text{CH}_2)_3\text{S}-\text{S}-\text{S}-(\text{CH}_2)_3\text{SO}_3\text{Na}$
- (b)  $\text{S}_2\text{Cl}_2 + 2\text{NaS}(\text{CH}_2)_3\text{SO}_3\text{Na} \rightarrow \text{NaO}_3\text{S}(\text{CH}_2)_3\text{S}-\text{S}-\text{S}-(\text{CH}_2)_3\text{SO}_3\text{Na}$
- (c)  $\text{ClCH}_2\text{CH}_2\text{Cl} + 2\text{NaSS}(\text{CH}_2)_3\text{SO}_3\text{Na} \rightarrow \text{NaO}_3\text{S}(\text{CH}_2)_3\text{SSCH}_2\text{CH}_2\text{SS}(\text{CH}_2)_3\text{SO}_3\text{Na}$
- (d)  $\text{ClCH}_2\text{CH}_2\text{Cl} + \text{NaSS}(\text{CH}_2)_3\text{SO}_3\text{Na} + \text{NaS}(\text{CH}_2)_3\text{SO}_3\text{Na} \rightarrow \text{NaO}_3\text{S}(\text{CH}_2)_3\text{SSCH}_2\text{CH}_2\text{S}(\text{CH}_2)_3\text{SO}_3\text{Na}$

15 Typical polysulfide compounds which may be employed according to the invention include the following compounds which are summarized in Table II. In the formula



M represents a sodium cation and R, R', and n are as indicated in Table II.

TABLE II  
Sulfonated Polysulfide Cooperating Brighteners of the Formula

| Additive | $\text{R}'$                                                                                                           | $n$ | $\text{R}$        |
|----------|-----------------------------------------------------------------------------------------------------------------------|-----|-------------------|
| S-1      |                                                                                                                       | 2   | $(\text{CH}_2)_3$ |
| S-2      |                                                                                                                       | 2   | $(\text{CH}_2)_3$ |
| S-3      |                                                                                                                       | 2   | $(\text{CH}_2)_3$ |
| S-4      |                                                                                                                       | 2   | $(\text{CH}_2)_3$ |
| S-5      |                                                                                                                       | 2   | $(\text{CH}_2)_3$ |
| S-6      |                                                                                                                       | 2   | $(\text{CH}_2)_3$ |
| S-7      |                                                                                                                       | 2   |                   |
| S-8      | $\text{NaO}_3\text{S}(\text{CH}_2)_2$                                                                                 | 2   | $(\text{CH}_2)_3$ |
| S-9      | $\text{NaO}_3\text{S}(\text{CH}_2)_3$                                                                                 | 2   | $(\text{CH}_2)_3$ |
| S-10     | $\text{NaO}_3\text{S}(\text{CH}_2)_4$                                                                                 | 2   | $(\text{CH}_2)_4$ |
| S-11     | $\text{NaO}_3\text{S}(\text{CH}_2)_3\text{Na}$ (or H)                                                                 | 4   | $(\text{CH}_2)_3$ |
| S-12     | $\text{NaO}_3\text{S}(\text{CH}_2)_3\text{S}_2(\text{CH}_2)_2$                                                        | 2   | $(\text{CH}_2)_3$ |
| S-13     | $\text{NaO}_3\text{S}(\text{CH}_2)_3\text{S}(\text{CH}_2)_2\text{CH}=\text{CHCH}_2$                                   | 2   | $(\text{CH}_2)_3$ |
| S-14     | $\text{NaO}_3\text{S}(\text{CH}_2)_3\text{S}(\text{CH}_2)_2\text{C}\equiv\text{CCH}_2$                                | 2   | $(\text{CH}_2)_3$ |
| S-15     | $\text{NaO}_3\text{S}(\text{CH}_2)_3\text{S}(\text{CH}_2)_2\text{CH}_2\text{C}_6\text{H}_4\text{C}\equiv\text{CCH}_2$ | 2   | $(\text{CH}_2)_3$ |
| S-16     | $\text{NaO}_3\text{S}(\text{CH}_2)_3\text{S}(\text{CH}_2)_2\text{CH}_2\text{CH}_2\text{CH}_2\text{CH}_2$              | 2   | $(\text{CH}_2)_3$ |
| S-17     | $\text{CH}_3\text{CH}_2\text{CH}_2\text{CH}_2$                                                                        | 2   | $(\text{CH}_2)_3$ |

| Additive | R'                                                                                | n R                                            |
|----------|-----------------------------------------------------------------------------------|------------------------------------------------|
| S-18     | $\text{H}_2\text{C}=\text{CHCH}_2$                                                | 2 $(\text{CH}_2)_3$                            |
| S-19     | $\text{HC}\equiv\text{CCH}_2$                                                     | 2 $(\text{CH}_2)_3$                            |
| S-20     |  | 2 $(\text{CH}_2)_3$                            |
| S-21     |  | 2 $(\text{CH}_2)_3$                            |
| S-22     | $\text{NaO}_2\text{SCH}_2\text{CH}(\text{OH})\text{CH}_2$                         | 2 $\text{CH}_2\text{CH}(\text{OH})\text{CH}_2$ |

The  $\text{R}'(\text{S})_n\text{Na}$  compound may be prepared by the reaction of  $\text{R}'\text{SNa}$  with sulfur if  $\text{R}'$  is an aromatic group (compounds S-1, S-2, S-3, S-4, S-5, S-20). A typical procedure is: To a methanol solution (150 ml.) containing sodium methoxide (0.1 m.) is added the  $\text{R}'\text{SH}$  (0.1 m.) compound. The mixture is stirred at room temperature until the compound has dissolved. Sulfur powder (0.1 m.) compound. The mixture is stirred at room temperature until all the sulfur is dissolved. Propanesultone (0.12 m.) is added to the stirred solution. Stirring is continued for 30 minutes, during which time a solid precipitates from the solution. Acetone (250 ml.) is then added to give additional solid, which is then filtered, washed with acetone, and dried.

Aliphatic  $\text{R}'(\text{S})_n\text{Na}$  compounds are prepared by reaction of  $\text{R}'\text{Q}$  with  $\text{Na}_2\text{S}_n$ , where  $\text{Q}$  is Cl, Br, I,  $-\text{OSO}_2\text{C}_6\text{H}_5$ ,  $-\text{OSO}_2\text{C}_6\text{H}_4\cdot\text{CH}_3$ ,  $-\text{OSO}_2\text{CH}_3$  (e.g., compounds S-17, S-18, S-19). A typical procedure is: To a stirred methanol solution (150 ml.) containing sodium disulfide (0.1 m.) is added dropwise a solution of  $\text{R}'\text{Q}$  (0.1 m.) in methanol (50 ml.) at room temperature. The reaction is slightly exothermic. After the addition is completed the mixture is stirred for 30 minutes. Propane sultone (0.12 m.), which may be dissolved in methanol (50 ml.), is added to the stirred mixture. During the addition of propane sultone a white solid usually precipitates from the solution. The mixture may be heated and stirred at 65° C. for 30 minutes and then cooled. Acetone is added and the solid is filtered and dried.

Compounds of the type of S-9, S-10, S-11, S-12 are prepared by the reaction of an alkali metal polysulfide ( $\text{Na}_2\text{S}_2$ ,  $\text{Na}_2\text{S}_4$ , etc.) with a sultone.

Compounds of the type of S-13, S-14, S-15, S-16 are prepared according to the reaction sequence:



(2)



Instead of sultones, haloalkane sulfonates, including, e.g.,  $\text{ClCH}_2\text{CHOHCH}_2\text{SO}_3\text{Na}$  (prepared by reaction of epichlorohydrin with sodium bisulfite), and in general compounds of the type  $\text{QRSO}_3\text{M}$ , may be used.

Some polysulfide compounds may also be prepared by the direct sulfonation of an organic polysulfide (e.g., S-7; or S-21 by sulfonation of S-20).

Symmetrical disulfides may be prepared by careful oxidation of compounds of the type  $\text{HSRSO}_3\text{Na}$ .

It is sometimes advantageous to prepare aqueous stock solutions of the sulfonated polysulfides containing small amounts of copper sulfate and/or sulfuric acid. Some precipitation may occur which is eliminated by filtration.

The sulfide compounds of the invention may be present in the copper bath in effective amount of about 0.001 g./l.-1.0 g./l., preferably 0.005 g./l.-0.2 g./l.

The heterocyclic cooperating additives of the invention may include heterocyclic compounds of the formulae:



The two formulae represent tautomeric forms wherein X is selected from the group consisting of



R'' is hydrogen or an alkyl, hydroxyalkyl, or aminoalkyl group of 1-6 carbon atoms and Y is a divalent organo group of 2-10 carbon atoms which forms a 5-6-membered cyclic ring structure with the group



or the group



Typical X groups may include groups of the formula



When Y is a divalent hydrocarbon group (including substituted hydrocarbon groups) Y may be a divalent alkylene group of 2-10 carbon atoms (such as an ethylene, propylene, etc., including alkyl-substituted divalent groups); Y may be an unsaturated group of 2-10 carbon atoms, and an amino- or hydroxy-substituted saturated or unsaturated hydrocarbon of 2-10 carbon atoms.

Typical heterocyclic compounds which may be employed according to the invention may include compounds of Table III wherein the groups X and Y of formulae (1) and (2) are as shown. The heterocyclic compounds may be employed in effective amounts, typically 0.5-10.0 mg./l. and preferably 0.7-4.0 mg./l. of total aqueous bath composition.

TABLE III.—HETERO CYCLIC COOPERATING AGENTS

| Additive | (X)          | (Y)                        | Structure                                                                            | Name                  |
|----------|--------------|----------------------------|--------------------------------------------------------------------------------------|-----------------------|
| H-1      | $-\text{S}-$ | $-\text{CH}_2\text{CH}_4-$ |  | 2-thiazolidinethione. |

| Additive  | (X)                                       | (Y)                                                            | Structure | Name                                                |
|-----------|-------------------------------------------|----------------------------------------------------------------|-----------|-----------------------------------------------------|
| H-2.....  | -S-                                       | CH <sub>3</sub><br>-CH <sub>2</sub> -CH-                       |           | 4-methyl-2-thiazolidinethione.                      |
| H-3.....  | -S-                                       | -CH=CH-                                                        |           | 2-thiazolethiol.                                    |
| H-4.....  | -S-                                       | -CH <sub>2</sub> CH <sub>2</sub> CH <sub>2</sub> -             |           | Tetrahydro-2H-1,3-thiazine-2-thione.                |
| H-5.....  | -O-                                       | -CH <sub>2</sub> CH <sub>2</sub> -                             |           | 2-oxazolidinethione.                                |
| H-6.....  | -NH-                                      | -CH <sub>2</sub> CH <sub>2</sub> -                             |           | 2-imidazolidinethione.                              |
| H-7.....  | -N-<br>CH <sub>2</sub> CH <sub>2</sub> OH | -CH <sub>2</sub> CH <sub>2</sub> -                             |           | 1-(2-hydroxyethyl)-2-imidazolidinethione.           |
| H-8.....  | -NH-                                      | -CH=CH-                                                        |           | 4-imidazoline-2-thione.                             |
| H-9.....  | -N-<br>CH <sub>3</sub>                    | -CH=CH-                                                        |           | 1-methyl-4-imidazoline-2-thione.                    |
| H-10..... | -NH-                                      | CH <sub>2</sub> CH <sub>2</sub> NH <sub>2</sub><br>-CH=C-      |           | 4-(2-aminoethyl)-2-imidazolethiol dihydrochloride.  |
| H-11..... | -N=                                       | =C-CH=CH-<br>CH <sub>3</sub>                                   |           | 4-methyl-2-pyrimidinethiol.                         |
| H-12..... | -NH-                                      | CH <sub>3</sub><br>-C=CH-C-<br>CH <sub>3</sub> CH <sub>3</sub> |           | 3,4-dihydro-4,4,6-trimethyl-2(1H)-pyrimidinethione. |
| H-13..... | -N=                                       | =C-CH=CH-<br>NH <sub>2</sub>                                   |           | 4-amino-2-pyrimidinethiol.                          |
| H-14..... | -N=                                       | =CH-CH=CH-<br>NH <sub>2</sub> NH <sub>2</sub>                  |           | 4,6-diamino-2-pyrimidinethiol.                      |
| H-15..... | -N-<br>H                                  | -CH <sub>2</sub> -CH <sub>2</sub> -CH <sub>2</sub> -           |           | Tetrahydro-2(1H)-pyrimidinethione.                  |

| Additive (X)  | (Y)                    | Structure | Name                            |
|---------------|------------------------|-----------|---------------------------------|
| H-16.....—N=  | =C—CH=CH—              |           | 4,6-dimethyl-2-pyrimidinethiol. |
| H-17.....—N=  | =CH—CH=CH—             |           | 2-pyrimidinethiol.              |
| H-18.....—NH— | =C—CH=CH—              |           | 2-thiouracil.                   |
| H-19.....—N—H | =C—CH <sub>2</sub> —C= |           | 2-thiobarbituric acid.          |

The heterocyclic cooperating additives of Table III may be obtained commercially or may be prepared as indicated herein. For example, compounds such as H-1 and H-4 may be prepared according to equation:



where  $r=2$  or  $3$  and  $Q'=\text{Cl, Br, I.}$

H-2 is prepared from the corresponding



This compound may also be prepared from propylene-imine and carbon disulfide.

H-3 is prepared from chloroacetaldehyde plus ammonium dithiocarbamate according to the equation:



H-5 may be prepared from ethanolamine and carbon disulfide, which by oxidation with iodine gives bis-(2-hydroxyethyl)-thiuram disulfide. Boiling of an aqueous suspension of this compound yields H-5.

Compounds such as H-1, H-2, H-4 may also be prepared by heating of the alkanolamine-carbon disulfide reaction product according to the equation:



Polyethers which may be used according to the process of the invention may have at least 5 ether oxygen atoms and include polyethers of the formulae:



60 where  $R'''$  is a monovalent radical such as H, alkyl, alkenyl, alkynyl, alkylaryl, arylalkyl or a heterocyclic radical; and  $R''''$  is a  $m$ -valent aliphatic, aromatic or heterocyclic radical;  $m=2$  to 100; and



where  $u$  and  $v=0$  to 4, but at least one of  $u$  or  $v$  must be greater than zero;  $r+s=6$  to 1000; and  $T=H$ , alkyl, benzyl,  $—SO_3M$ ,  $—C_uH_{2u}SO_3M$ ,  $—PO_3H_2$ .

Suitable polyethers which may be used according to the invention include polyethers set forth in Table IV. The polyether additives may be employed in effective amounts, typically 0.005-10.0 g./l. and preferably 0.1-1.0 g./l. of total aqueous bath composition.

TABLE IV. COOPERATING POLYESTERS

## Additive

 $m+n=30$ P-2. Formula 3 wherein  $m+n=15$ P-3. Formula 3 wherein  $m+n=10$ P-5. Formula 4 wherein  $x=30$ P-6. Formula 4 wherein  $x=40$ 

wherein  $m$  = about 12-15  
 $n$  = about 1-2

The chloride ion content of the aqueous copper plating bath compositions of the invention may be at least about 0.5 mg./l. and typically from 1.0 mg./l. to 500 mg./l. of aqueous copper plating bath. Good results may be obtained using a chloride ion concentration of from about 4 mg./l. to 60 mg./l. of aqueous copper plating bath composition, and preferably a chloride ion concentration of from 20 mg./l. to 60 mg./l. of aqueous copper plating solution.

Other optional additives used were the following dispersing agents:

For the purpose of providing those skilled-in-the-art with a better understanding of this invention, the following examples are set forth.

35 In these examples the aqueous copper plating bath contains:

$\text{CuSO}_4 \cdot 5\text{H}_2\text{O}$ , 220 g./l.

$\text{H}_2\text{SO}_4$ , 60 g./l

Chloride ion, 0.03-0.04 g./l.

The plating experiments were performed in a Hull Cell containing 250 ml. of this acid copper sulfate bath. The

TABLE V

| Additives |                                           |
|-----------|-------------------------------------------|
| D-1.....  |                                           |
| D-2.....  |                                           |
| D-3.....  |                                           |
|           | where $n=3$ to $6$                        |
| D-4.....  |                                           |
|           | $n+m=1-2$ and preferably $n=0$ when $m=1$ |
| D-5.....  |                                           |

wherein each  $n$  is an integer 4-12 (preferably 4-8) and each of  $M_1$  and  $M_2$  is an alkali metal (preferably Na or K) or a hydrogen atom.

Hull Cell allows one to observe the appearance of the deposit over a wide current density range. In order to judge the degree of leveling the polished brass panels used for these plating tests were scratched with 4/0 emery polishing paper over a horizontal band of about 10 mm. width. The plating temperature used in these experiments was the ambient room temperature (24-30° C.), unless otherwise stated. The total current was 2 amperes and the plating time 10 minutes. Air agitation or mechanical agitation with an oscillating paddle was used as specified in Table VI. The sulfonated polysulfide compounds used are described in Table II, the heterocyclic compounds in Table III, and the polyethers in Table IV.

For convenience, the results shown in Table VI are classified according to (1) the width of the lustrous current density range (semi-bright to bright) and according to (2) the degree of leveling under the indicated experimental conditions (i.e., a 250-ml. Hull Cell, 2 amperes current, and a ten-minute plating time on a metal strip having a band uniformly scratched with 4/0 grit emery paper).

Each property in groups (1) and (2) is independently measured as "poor," "fair," "good," and "very good" as follows:

|    | Additives            | Amount, g./l.                   | Type of agitation | Results    |
|----|----------------------|---------------------------------|-------------------|------------|
| 5  | { S-1<br>P-12<br>H-1 | { 0.02<br>0.1<br>0.001          | Air.....          | Very good. |
|    | { S-1<br>P-13<br>H-1 | { 0.02<br>0.20<br>0.02          | Air.....          | Poor.      |
| 10 | { S-1<br>P-13<br>H-1 | { 0.20<br>0.001<br>0.02         | Air.....          | Very good. |
|    | { S-2<br>P-1<br>S-2  | { 0.03<br>1.00<br>0.03          | Air.....          | Poor.      |
|    | { P-1<br>H-1<br>H-7  | { 1.00<br>0.4<br>0.00075        | Air.....          | Do.        |
|    | { S-2<br>P-1<br>H-7  | { 0.03<br>1.00<br>0.00075       | Air.....          | Good.      |
|    | { P-1<br>H-1<br>H-7  | { 0.00075<br>0.00075<br>0.00075 | Air.....          | Do.        |
|    | { S-2<br>P-1<br>H-7  | { 0.03<br>1.00<br>0.00075       | Air.....          | Excellent. |
|    | { S-4<br>P-1<br>S-4  | { 0.03<br>1.00<br>0.03          | Air.....          | Poor.      |
|    | { P-1<br>H-1<br>H-7  | { 1.00<br>0.00075<br>0.00075    | Air.....          | Good.      |
| 25 | { S-5<br>P-1<br>S-5  | { 0.03<br>1.00<br>0.03          | Air.....          | Poor.      |
|    | { P-1<br>H-1<br>H-7  | { 1.00<br>0.00075<br>0.00075    | Air.....          | Very good. |

| Property (1) |                                                                     | Property (2) |                                                                                                                    |
|--------------|---------------------------------------------------------------------|--------------|--------------------------------------------------------------------------------------------------------------------|
| Rating       | Width of lustrous current density range                             | Rating       | Degree of leveling                                                                                                 |
| Poor         | Less than one half of length of test panel                          | Poor         | No visual change in original roughness of scratched band                                                           |
| Fair         | More than one half and less than two thirds of length of test panel | Fair         | Noticeable decrease in roughness, but scratches still visible.                                                     |
| Good         | More than two thirds but less than entire length of test panel      | Good         | Roughness decreased and portions of scratches completely level.                                                    |
| Very good    | Entire length of test panel is lustrous                             | Very good    | Scratches on the portion of the panel having a current density greater than 2.5 a./s.d. are practically invisible. |

The combination of the panel ratings given with respect to width of lustrous current density range and degree of leveling determine the final classification set forth in the "Results" column of Table VI according to the following:

| Results   | Definition                                                                                                                                               |
|-----------|----------------------------------------------------------------------------------------------------------------------------------------------------------|
| Excellent | Very good leveling and very good bright current density range.                                                                                           |
| Very good | Very good leveling and good bright current density range.                                                                                                |
| Good      | Good to very good leveling and good to very good semi-bright current density range or: good leveling and good to very good bright current density range. |
| Poor      | Poor leveling and/or poor lustrous current density range.                                                                                                |
| Fair      | All intermediate panels not otherwise classified.                                                                                                        |

TABLE VI

| Example No.: | Additives                  | Amount, g./l.                         | Type of agitation | Results    |
|--------------|----------------------------|---------------------------------------|-------------------|------------|
| 1            | { S-1<br>P-1               | { 0.03<br>1.00                        | Air.....          | Poor.      |
| 2            | { P-1<br>H-1               | { 1.00<br>0.001                       | Air.....          | Good.      |
| 3            | { P-1<br>H-1<br>D-1        | { 1.00<br>0.001<br>0.40               | Air.....          | Excellent. |
| 4            | { P-1<br>H-1<br>H-7        | { 1.00<br>0.000625<br>0.000625        | Air.....          | Good.      |
| 5            | { P-1<br>H-1<br>H-7<br>D-1 | { 1.00<br>0.000625<br>0.000625<br>0.4 | Air.....          | Excellent. |
| 6            | { S-1<br>P-8               | { 0.02<br>1.00                        | Mechanical.....   | Poor.      |
| 7            | { S-1<br>P-8<br>H-1        | { 0.02<br>1.00<br>0.001               | do.....           | Very good. |
| 8            | { S-1<br>P-11              | { 0.02<br>0.1                         | Air.....          | Poor.      |
| 9            | { P-11<br>H-1              | { 0.02<br>0.001                       | Air.....          | Fair.      |
| 10           | { S-1<br>P-12              | { 0.02<br>0.1                         | Air.....          | Poor.      |
| 40           | { S-5<br>P-1<br>H-7<br>D-1 | { 0.03<br>1.00<br>0.4<br>0.00075      | Air.....          | Excellent. |
| 45           | { S-6<br>P-1<br>S-6        | { 0.03<br>1.00<br>0.03                | Air.....          | Poor.      |
|              | { P-1<br>H-1<br>H-7        | { 1.00<br>0.00075<br>0.00075          | Air.....          | Good.      |
|              | { S-6<br>P-1<br>H-7        | { 0.03<br>1.00<br>0.00075             | Air.....          | Very good. |
| 50           | { H-1<br>D-1               | { 0.00075<br>0.4                      | Mechanical.....   | Poor.      |
|              | { S-7<br>S-7               | { 0.05<br>0.20                        | do.....           | Do.        |
|              | { S-7<br>P-4               | { 0.20<br>0.01                        | do.....           | Fair.      |
|              | { S-7<br>P-4<br>H-1        | { 0.20<br>0.01<br>0.001               | do.....           | Good.      |
|              | { S-7<br>P-5               | { 0.05<br>0.50                        | do.....           | Poor.      |
|              | { S-7<br>P-5               | { 0.05<br>0.50                        | do.....           | Good.      |
|              | { S-7<br>P-5<br>H-1        | { 0.20<br>0.20<br>0.001               | do.....           | Poor.      |
|              | { S-7<br>P-5<br>H-1        | { 0.20<br>0.20<br>0.001               | do.....           | Good.      |
|              | { S-7<br>P-12              | { 0.5<br>0.05                         | do.....           | Poor.      |
|              | { S-7<br>P-12              | { 0.5<br>0.05                         | do.....           | Good.      |
| 60           | { S-7<br>P-1<br>H-1        | { 0.20<br>1.00<br>0.001               | do.....           | Poor.      |
| 65           | { S-7<br>P-1<br>S-7        | { 0.20<br>1.00<br>0.20                | Air.....          | Poor.      |
|              | { P-1<br>H-1<br>H-7        | { 1.00<br>0.00075<br>0.00075          | Air.....          | Very good. |
| 70           | { P-1<br>H-1<br>H-7<br>D-1 | { 1.00<br>0.00075<br>0.00075<br>0.4   | Air.....          | Do.        |
|              | { S-8<br>P-1<br>S-8        | { 0.02<br>1.00<br>0.02                | Air.....          | Poor.      |
|              | { S-8<br>P-1<br>H-1        | { 0.02<br>1.00<br>0.001               | Air.....          | Fair.      |
| 75           | { P-1<br>H-1               | { 1.00<br>0.001                       | Air.....          | Good.      |

|    | Additives                 | Amount, g./l.                        | Type of agitation | Results            |    | Additives | Amount, g./l.         | Type of agitation      | Results      |            |
|----|---------------------------|--------------------------------------|-------------------|--------------------|----|-----------|-----------------------|------------------------|--------------|------------|
| 41 | {S-8<br>P-1<br>H-1<br>D-1 | 0.02<br>1.00<br>0.001<br>0.2         | Air.....          | Good.              | 5  | 76        | {S-13<br>P-12         | Air.....               | Poor.        |            |
| 42 | {S-9<br>P-1               | 0.02<br>1.00                         | Air.....          | Poor.              |    | 77        | {S-13<br>P-12<br>H-1  | 0.01<br>0.25<br>0.001  | Air.....     | Good.      |
| 43 | {S-9<br>P-1<br>H-1        | 0.02<br>1.00<br>0.001                | Air.....          | Good.              |    | 78        | {S-15<br>P-14         | 0.01<br>0.50           | Air.....     | Poor.      |
| 44 | {S-9<br>P-1<br>H-1<br>D-2 | 0.02<br>1.00<br>0.001<br>0.40        | Air.....          | Excellent.         | 10 | 79        | {S-15<br>P-14<br>H-1  | 0.01<br>0.50<br>0.001  | Air.....     | Excellent. |
| 45 | {S-9<br>P-1<br>H-1<br>H-7 | 0.02<br>1.00<br>0.000625<br>0.000625 | Air.....          | Good.              |    | 80        | {S-16<br>P-1          | 0.005<br>1.00          | Air.....     | Fair.      |
| 46 | {H-1<br>H-7<br>D-1        | 0.000625<br>0.000625<br>0.40         | Air.....          | Excellent.         | 15 | 81        | {S-16<br>P-1<br>H-12  | 0.005<br>1.00<br>0.001 | Air.....     | Good.      |
| 47 | {S-9<br>P-1<br>H-3        | 0.02<br>1.00<br>0.001-0.002          | Air.....          | Good.              | 20 | 82        | {H-12<br>D-1          | 0.4<br>0.02            | Air.....     | Very good. |
| 48 | {P-1<br>H-4<br>S-9        | 1.00<br>0.001<br>0.02                | Air.....          | Very good.         |    | 83        | {S-17<br>P-10         | 0.02<br>1.00           | Air.....     | Poor.      |
| 49 | {P-1<br>H-4<br>D-1        | 1.00<br>0.001<br>0.2                 | Air.....          | Excellent.         |    | 84        | {S-17<br>P-10<br>H-14 | 0.02<br>1.00<br>0.001  | Air.....     | Very good. |
| 50 | {S-9<br>P-1<br>H-5        | 0.02<br>1.00<br>0.002                | Air.....          | Very good.         | 25 | 85        | {S-18<br>P-8          | 0.03<br>1.00           | Mechanical.. | Poor.      |
| 51 | {P-1<br>H-5<br>D-1        | 1.00<br>0.002<br>0.20                | Air.....          | Excellent.         |    | 86        | {S-18<br>P-8<br>H-1   | 0.03<br>1.00<br>0.001  | do.....      | Very good. |
| 52 | {S-9<br>P-1<br>H-6        | 0.02<br>1.00<br>0.002                | Air.....          | Good.              | 30 | 87        | {S-19<br>P-10         | 0.02<br>1.00           | Air.....     | Fair.      |
| 53 | {S-9<br>P-1<br>H-7        | 0.02<br>1.00<br>0.002                | Air.....          | Good.              |    | 88        | {S-19<br>P-10<br>H-1  | 0.02<br>1.00<br>0.0012 | Air.....     | Very good. |
| 54 | {S-9<br>P-1<br>H-7<br>D-1 | 0.02<br>1.00<br>0.4                  | Air.....          | Do.                | 35 | 89        | {S-19<br>P-14         | 0.03<br>1.00           | Air.....     | Fair.      |
| 55 | {S-9<br>P-1<br>H-9        | 0.02<br>1.00<br>0.002                | Air.....          | Very good.         |    | 90        | {S-19<br>P-14<br>H-1  | 0.03<br>1.00<br>0.001  | Air.....     | Very good. |
| 56 | {P-1<br>H-12              | 1.00<br>0.001                        | Air.....          | Do.                | 40 | 91        | {S-20<br>P-12         | 0.02<br>0.50           | Air.....     | Fair.      |
| 57 | {P-1<br>H-13              | 1.00<br>0.000625                     | Air.....          | Do.                |    | 92        | {S-20<br>P-12<br>H-1  | 0.02<br>0.50<br>0.001  | Air.....     | Excellent. |
| 58 | {P-1<br>H-14              | 1.00<br>0.001                        | Air.....          | Good.              |    | 93        | {S-21<br>P-14         | 0.03<br>0.50           | Air.....     | Fair.      |
| 59 | {P-1<br>H-15              | 1.00<br>0.0006                       | Air.....          | Do.                | 50 | 94        | {S-21<br>P-14<br>H-1  | 0.30<br>0.50<br>0.001  | Air.....     | Very good. |
| 60 | {P-1<br>H-16              | 1.00<br>0.0006                       | Air.....          | Do.                |    | 95        | {S-22<br>P-12         | 0.04<br>0.50           | Air.....     | Fair.      |
| 61 | {S-9<br>P-1<br>H-18       | 0.02<br>1.00<br>0.002                | Air.....          | Do.                |    | 96        | {S-22<br>P-12<br>H-1  | 0.04<br>0.50<br>0.001  | Air.....     | Very good. |
| 62 | {S-9<br>P-5               | 0.02<br>0.25                         | Mechanical..      | Poor.              |    |           |                       |                        |              |            |
| 63 | {P-5<br>H-1               | 0.25<br>0.001                        | do.....           | Excellent.         |    |           |                       |                        |              |            |
| 64 | {P-7<br>H-1               | 0.25<br>0.001                        | do.....           | Do.                |    |           |                       |                        |              |            |
| 65 | {S-9<br>P-12              | 0.02<br>0.10                         | Air.....          | Poor.              |    |           |                       |                        |              |            |
| 66 | {S-9<br>P-12              | 0.02<br>0.10                         | Air.....          | Very good.         |    |           |                       |                        |              |            |
| 67 | {S-9<br>P-13              | 0.01<br>0.1                          | Air.....          | Fair.              | 60 |           |                       |                        |              |            |
| 68 | {P-13<br>H-1              | 0.01<br>0.00125                      | Air.....          | Excellent.         |    |           |                       |                        |              |            |
| 69 | {S-9<br>P-13              | 0.01<br>1.00                         | Air.....          | Poor. <sup>1</sup> |    |           |                       |                        |              |            |
| 70 | {S-9<br>P-13<br>H-1       | 0.01<br>1.00<br>0.003                | Air.....          | Good. <sup>1</sup> | 65 |           |                       |                        |              |            |
| 71 | {S-10<br>P-1              | 0.01<br>1.00                         | Air.....          | Poor.              |    |           |                       |                        |              |            |
| 72 | {S-10<br>P-1              | 0.01<br>1.00                         | Air.....          | Very good.         |    |           |                       |                        |              |            |
| 73 | {S-11<br>P-1              | 0.02<br>1.00                         | Air.....          | Poor.              | 70 |           |                       |                        |              |            |
| 74 | {S-11<br>P-1<br>H-7       | 0.02<br>1.00<br>0.002                | Air.....          | Good.              |    |           |                       |                        |              |            |
| 75 | {P-1<br>H-7<br>D-1        | 1.00<br>0.002<br>0.4                 | Air.....          | Do.                | 75 |           |                       |                        |              |            |

<sup>1</sup> At 46° C.

As can be readily seen from above examples of Table VI, the combination of an aromatic or aliphatic polysulfide sulfonate (compounds S of Table II) and of a polyether (such as the compounds P of Table IV) generally gives matte deposits in the low and medium current density range and/or the degree of leveling over a rough substrate is low.

50 Addition of at least one heterocyclic compound (H) of the type described in Table III to the combination of S and P very strongly increases leveling and widens the bright current density range toward lower current densities. The addition of a compound (H) often increases also the intensity of brightness.

55 Results similar to those reported in Table VI (wherein a copper sulfate bath was used) may be obtained with a fluoroborate bath using higher current densities and somewhat higher concentrations of the heterocyclic compounds, (H). For instance, using a fluoroborate electrolyte containing:

$\text{Cu}(\text{BF}_4)_2$ , 224 g./l.  
 $\text{HBF}_4$ , 3.5 g./l.  
 $\text{H}_3\text{BO}_3$ , 15.0 g./l.  
 $\text{Cl}^-$ , 0.03 g./l.

The simultaneous addition of:

S-9, 0.02 g./l.  
P-1, 1.00 g./l.  
H-1, 0.001 g./l.  
H-7, 0.001 g./l.

gave a bright, strongly leveled copper deposit in an air agitated Hull Cell (250 ml.) at 5 amperes total current in 5 minutes, up to the high current density end of the cell (about 30 a.s.d.).

## 21

Although this invention has been illustrated by reference to specific embodiments, modifications thereof which are clearly within the scope of the invention will be apparent to those skilled-in-the-art.

What is claimed is:

1. A process for electrodepositing bright, strongly leveled, ductile copper from an aqueous acidic copper plating bath containing chloride ions and at least one member from each of the following groups:

(1) a polysulfide compound of the formula



in effective amount of 0.001 g./l.-1.0 g./l.

(2) a heterocyclic compound of the formula



and/or tautomers thereof in effective amount 0.5-10.0 mg./l.; and

(3) a polyether, containing at least 5 ether oxygen atoms per molecule in effective amount of 0.005-10.0 g./l.

wherein each R is independently a divalent aliphatic or aromatic non-heterocyclic group of 1-10 carbon atoms; R' is hydrogen, a metal cation, a monovalent aliphatic or aromatic organo group of 1-20 carbon atoms, or the groups  $-R-SO_3 M$  or  $-R-(S)_q-RSO_3 M$  wherein q is an integer 2-5; M is a cation;



R'' is hydrogen or an alkyl, hydroxyalkyl or aminoalkyl group of 1-6 carbon atoms; Y is a divalent organo group of 1-10 carbon atoms which forms a 5-6 membered cyclic ring structure with the group



and n is an integer 2-5 inclusive.

2. The process as claimed in claim 1 wherein n is an integer 2-4.

3. The process as claimed in claim 1 wherein n is an integer 2-4, R' is an aromatic group, and R is a polymethylene group.

4. A process as claimed in claim 1 wherein the polysulfide compound is of the formula



in which R' is  $NaO_3 S(CH_2)_3$ ; n is 2; and R is  $(CH_2)_3$ .

5. A process as claimed in claim 1 wherein the polysulfide compound is of the formula



in which R' is  $NaO_3 S(CH_2)_3 S_2 (CH_2)_2$ ; n is 2; and R is  $(CH_2)_3$ .

6. A process as claimed in claim 1 wherein the polysulfide compound is of the formula



in which R' is  $NaO_3 S(CH_2)_3 S_2 CH_2 CH=CHCH_2$ ; n is 2; and R is  $(CH_2)_3$ .

7. A process as claimed in claim 1 wherein the polysulfide compound is of the formula



in which R' is  $NaO_3 S(CH_2)_3 S_2 CH_2 C=CCH_2$ ; n is 2; and R is  $(CH_2)_3$ .

## 22

8. A process as claimed in claim 1 wherein the polysulfide compound is of the formula



in which R' is  $NaO_3 S(CH_2)_3 S_2 (CH_2)_5$ ; n is 2; and R is  $(CH_2)_3$ .

9. A process as claimed in claim 1 wherein the polysulfide compound is of the formula



in which R' is  $H_2 C=CHCH_2$ ; n is 2; and R is  $(CH_2)_3$ .

10. A process as claimed in claim 1 wherein the polysulfide compound is of the formula



in which R' is  $HC=CCH_2$ ; n is 2; and R is  $(CH_2)_3$ .

11. A process as claimed in claim 1 wherein the polysulfide compound is of the formula



in which R' is  $NaO_3 SCH_2 CH(OH)CH_2$ ; n is 2; and R is  $CH_2 CH(OH)CH_2$ .

12. A process as claimed in claim 1 wherein X is  $-S-$ .

13. A process as claimed in claim 1 wherein X is  $-O-$ .

14. A process as claimed in claim 1 wherein X is



15. A process as claimed in claim 1 wherein X is



16. A process as claimed in claim 1 wherein Y is  $-CH_2 CH_2 -$ .

17. A process as claimed in claim 1 wherein the chloride ion concentration is at least 0.5 mg./l. of total aqueous bath composition.

18. A process as claimed in claim 1 wherein the chloride ion concentration is 1-500 mg./l. of total aqueous bath composition.

19. A process as claimed in claim 1 wherein the polyether is



m+n=30, and wherein the process is carried out in the presence of a dispersing agent of the formula



20. A process as claimed in claim 1 wherein the polyether is



wherein x is about 3 and y is about 3-4.

21. A process as claimed in claim 1 wherein the polyether contains oxypropylene and oxyethylene groups.

22. A composition for electrodepositing bright, strongly leveled, ductile copper which comprises an aqueous acidic copper plating bath containing chloride ions and at least one member from each of the following groups:

(1) a polysulfide compound of the formula



in effective amount of 0.01 g./l.-1.0 g./l.  
(2) a heterocyclic compound of the formula



and/or tautomers thereof in effective amount of 0.5-10.0 mg./l.; and

(3) a polyether, containing at least 5 ether oxygen atoms per molecule in effective amount of 0.005-10.0 g./l.

wherein each R is independently a divalent aliphatic or aromatic non-heterocyclic group of 1-10 carbon atoms; R' is hydrogen, a metal cation, a monovalent aliphatic or aromatic organo group of 1-20 carbon atoms, or the groups  $-R-SO_3M$  or  $-R-(S)_q-RSO_3$  wherein q is an integer 2-5; M is a cation;



R'' is hydrogen or an alkyl, hydroxyalkyl or aminoalkyl group of 1-6 carbon atoms; Y is a divalent organo group of 1-10 carbon atoms which forms a 5-6 membered cyclic ring structure with the group



and n is an integer 2-5 inclusive.

23. A composition as claimed in claim 22 wherein n is an integer 2-4.

24. A composition as claimed in claim 22 wherein n is an integer 2-4, R' is an aromatic group, and R is a polymethylene group.

25. A composition as claimed in claim 22 wherein X is  $-S-$ .

26. A composition as claimed in claim 22 wherein X is  $-O-$ .

27. A composition as claimed in claim 22 wherein X is



28. A composition as claimed in claim 22 wherein X is



5 29. A composition as claimed in claim 22 wherein Y is  $-CH_2CH_2-$ .

30. A composition as claimed in claim 22 wherein the chloride ion concentration is at least 0.5 mg./l. of total aqueous bath composition.

10 31. A composition as claimed in claim 22 wherein the chloride ion concentration is 1-500 mg./l. of total aqueous bath composition.

32. A composition as claimed in claim 22 wherein the polyether is



20 25  $m+n=30$ , and containing a dispersing agent of the formula



30 33. A composition as claimed in claim 22 wherein the polyether is



35 wherein x is about 3 and y is about 3-4.

#### References Cited

#### UNITED STATES PATENTS

|           |         |               |       |        |
|-----------|---------|---------------|-------|--------|
| 2,663,684 | 12/1953 | Pierce        | ----- | 204-52 |
| 2,700,020 | 1/1955  | Pierce        | ----- | 204-52 |
| 2,840,518 | 6/1958  | Condon        | ----- | 204-52 |
| 3,267,010 | 8/1966  | Creutz et al. | ----- | 204-52 |
| 3,288,690 | 11/1966 | Creutz et al. | ----- | 204-52 |
| 3,328,273 | 6/1967  | Creutz et al. | ----- | 204-52 |

GERALD L. KAPLAN, Primary Examiner